

## UNITED STATES PATENT OFFICE

GIUSEPPE BIANCO, OF TURIN, ITALY

## ELECTROLYTIC ZINC BATH

No Drawing.

Application filed April 20, 1927. Serial No. 185,365.

This invention relates to a novel electrolytic zinc bath by means of which iron, steel or cast iron articles can be coated with a perfectly uniform, smooth and compact layer 5 of high grade zinc.

The purpose of the present invention is to provide an electrolytic bath of great stability which shall be automatically regenerated without adding any fresh ingredients thereto 10 and is therefore capable of working in a continuous manner and for an unlimited period of time without necessitating any regenerating process like electrolytic baths known heretofore.

15 An important feature of this invention consists in the fact that the zinc coated articles are absolutely free from any spongy zones which, as is well known, occur quite often in the zinc coated articles obtained with 20 the usual electrolytic processes and are always the source of corruptions due to the natural agents.

A further feature of this electrolytic bath is that it allows to regulate at will the depth 25 of the layer deposited and to accelerate the zinc deposition by employing high current intensities, without altering in the least the structure of the metal and the adherence of the zinc layer.

30 In known zinc baths, the electrolyte is generally made of zinc sulphate and conductive salts dissolved in water; these solutions have the drawback that they are not perfectly homogeneous and are rapidly exhausted.

35 Moreover, owing to the large quantity of hydrogen set off at the cathode with the use of those known electrolytes the production of a compact deposit free from spongy zones on large surfaces meets with serious difficulties.

40 This invention completely obviates the above mentioned drawbacks by employing zinc in combination with mercury, sulphuric acid, phosphoric acid, conductive salts and distilled water.

The solution is prepared as follows: I first make by melting zinc and mercury to an amalgam in the proportions hereinafter described which, by lowering the melting point 45 of zinc, makes it possible to deprive the zinc

of any impurity therein contained that produces objectionable disturbances during the electrodeposition of the zinc. The molten amalgam thus purified is successively projected into a refrigerating liquid thereby 55 obtaining the special porous form mentioned above and containing both metals in the following proportions in weight, zinc 100 to 200, mercury 1 to 15.

The product is dissolved in distilled water 60 to which sulphuric acid, phosphoric acid and the conductive salts have been previously added. This mass rapidly reacts developing heat and when the reaction is completed the solution is clarified and filtered and 65 the liquid ready for use is obtained. I also obtain the said porous zinc by melting it in the presence of iron and projecting it into a refrigerating liquid as explained and in this case successively adding mercury together 70 with the other above mentioned substances during formation of the mixture.

The presence of phosphorus which, as is well known, has a strong affinity with nascent hydrogen, makes it possible to completely 75 eliminate during the electrodeposition, the spongy zones on the surfaces of iron, steel or other metal coated with zinc. In fact phosphorus, added in the form of an elementary body or of a chemical compound, during 80 the reaction of the various component substances gives to the solution a colloidal form which prevents the formation of free hydrogen at the cathode by binding nascent hydrogen. 85

The solution that has practically given the best results is obtained with the following substances in the proportions indicated:

|                                          | Parts by weight | 90 |
|------------------------------------------|-----------------|----|
| Zinc-mercury amalgam                     | 101 to 215      |    |
| Sulphuric acid                           | 125 to 275      |    |
| Double sulphate of iron and alu-<br>mina | 15 to 40        |    |
| Phosphoric acid                          | 5 to 15         | 95 |
| Sodium and potassium hydrox-<br>ide      | 5 to 15         |    |
| Distilled water                          | 1000            |    |

The secondary constituents of the electro-  
lyte can also be used in the form of simple 100

or double compounds corresponding to the acids and bases mentioned above.

What I claim is:

1. An electrolytic zinc bath comprising a zinc amalgam, phosphoric acid combined with an alkali metal, sulphuric acid, aluminium hydroxide, and water.

2. An electrolytic zinc bath containing:

|                                  | Parts by weight |
|----------------------------------|-----------------|
| 10 Zinc-mercury amalgam-----     | 101 to 215      |
| Sulphuric acid -----             | 125 to 275      |
| Mixed sulphates of iron and alu- |                 |
| mina-----                        | 15 to 40        |
| Phosphoric acid-----             | 5 to 10         |
| 15 Alkali metal hydroxide-----   | 5 to 15         |
| Distilled water -----            | 1000            |

3. An electrolytic zinc bath comprising a mixture of zinc amalgam, sulphuric acid, alkali metal hydroxide and a phosphorus containing substance that will react in the solution to bind hydrogen at the cathode.

4. An electrolytic zinc bath comprising a zinc amalgam, alkali metal hydroxide, phosphoric acid, sulphuric acid and water.

5. An electrolytic zinc bath comprising a zinc amalgam, alkali metal hydroxide, aluminium hydroxide, a phosphoric acid, sulphuric acid and water.

30 In testimony that I claim the foregoing as my invention, I have signed my name.

GIUSEPPE BIANCO.